



US005571649A

**United States Patent** [19]**Mishra et al.****Patent Number:** **5,571,649****Date of Patent:** **Nov. 5, 1996****[54] ELECTROPHOTOGRAPHIC IMAGING MEMBER WITH IMPROVED UNDERLAYER**

[75] Inventors: **Satchidanand Mishra; Robert C. U. Yu, both of Webster; Kathleen M. Carmichael, Williamson; Edward F. Grabowski, Webster; Anthony M. Horgan, Pittsford; William W. Limburg, Penfield; Sharon E. Normandin, Macedon; Damodar M. Pai, Fairport; Richard L. Post, Penfield; Donald P. Sullivan, Rochester; Donald C. VonHoene, Fairport, all of N.Y.**

[73] Assignee: **Xerox Corporation**, Stamford, Conn.

[21] Appl. No.: **587,121**

[22] Filed: **Jan. 11, 1996**

[51] Int. Cl.<sup>6</sup> ..... **G03G 5/14**

[52] U.S. Cl. ..... **430/59**; 430/65; 430/96

[58] Field of Search ..... 430/58, 59, 64, 430/65, 96, 128

**[56] References Cited****U.S. PATENT DOCUMENTS**

4,464,450 8/1984 Teuschu ..... 430/59  
4,587,189 5/1986 Hor et al. ..... 430/59  
4,588,667 5/1986 Jones et al. ..... 430/73

|           |         |                     |        |
|-----------|---------|---------------------|--------|
| 4,780,385 | 10/1988 | Wieloch et al. .... | 430/58 |
| 4,786,570 | 11/1988 | Yu et al. ....      | 430/58 |
| 4,925,760 | 5/1990  | Baranyi et al. .... | 430/76 |
| 4,943,508 | 7/1990  | Yu ....             | 430/58 |
| 5,019,473 | 5/1991  | Nguyen et al. ....  | 430/58 |
| 5,322,755 | 6/1994  | Allen et al. ....   | 430/96 |
| 5,418,100 | 5/1995  | Yu ....             | 430/58 |

*Primary Examiner*—John Goodrow

**[57] ABSTRACT**

An electrophotographic imaging member comprising a support substrate having a two layered electrically conductive ground plane layer comprising a layer comprising zirconium over a layer comprising titanium, a hole blocking layer, an adhesive layer comprising a polymer blend comprising a carbazole polymer and a film forming thermoplastic resin selected from the group consisting of copolyester, polyarylate and polyurethane in contiguous contact with the hole blocking layer, a charge generation layer comprising perylene or a phthalocyanine pigment particles dispersed in a polycarbonate film forming binder in contiguous contact with the adhesive layer, and a hole transport layer, the hole transport layer being substantially non-absorbing in the spectral region at which the charge generation layer generates and injects photogenerated holes but being capable of supporting the injection of photogenerated holes from the charge generation layer and transporting the holes through the charge transport layer.

**28 Claims, No Drawings**

**ELECTROPHOTOGRAPHIC IMAGING  
MEMBER WITH IMPROVED UNDERLAYER**

**BACKGROUND OF THE INVENTION**

This invention relates in general to electrophotography and more specifically, to an improved electrophotographic imaging member having an improved adhesive layer.

In the art of electrophotography, an electrophotographic plate comprising a photoconductive insulating layer on a conductive layer is imaged by first uniformly electrostatically charging surface of the photoconductive insulating layer. The plate is then exposed to a pattern of activating electromagnetic radiation such as light, which selectively dissipates the charge in the illuminated areas of the photoconductive insulating layer while leaving behind an electrostatic latent image in the non-illuminated areas. This electrostatic latent image may then be developed to form a visible image by depositing finely divided electroscopic toner particles on the surface of the photoconductive insulating layer. The resulting visible toner image can be transferred to a suitable receiving member such as paper. This imaging process may be repeated many times with reusable photoconductive insulating layers.

Electrophotographic imaging members are usually multilayered photoreceptors that comprise a substrate support, an electrically conductive layer, an optional hole blocking layer, an adhesive layer, a charge generating layer, and a charge transport layer in either a flexible belt form or a rigid drum configuration. For most multilayered flexible photoreceptor belts, an anti-curl layer is usually employed on the back side of the substrate support, opposite to the side of the electrically active layers, to render the desired photoreceptor flatness. One type of multilayered photoreceptor comprises a layer of finely divided particles of a photoconductive inorganic compound dispersed in an electrically insulating organic resin binder. U.S. Pat. No. 4,265,990 discloses a layered photoreceptor having separate charge generating (photogenerating) and charge transport layers. The charge generating layer is capable of photogenerating holes and injecting the photogenerated holes into the charge transport layer. The photogenerating layer utilized in multilayered photoreceptors include, for example, inorganic photoconductive particles or organic photoconductive particles dispersed in a film forming polymeric binder. Inorganic or organic photoconductive material may be formed as a continuous, homogeneous photogenerating layer. Many suitable photogenerating materials known in the art can be utilized, if desired.

As more advanced, higher speed electrophotographic copiers, duplicators and printers were developed, degradation of image quality was encountered during extended cycling. Moreover, complex, highly sophisticated, duplicating and printing systems employed flexible photoreceptor belts, operating at very high speeds, have also placed stringent mechanical requirements and narrow operating limits as well on photoreceptors. For example, the layers of many modern multilayered photoreceptor belt must be highly flexible, adhere well to each other, and exhibit predictable electrical characteristics within narrow operating limits to provide excellent toner images over many thousands of cycles.

A typical prior art multilayered flexible photoreceptor configuration comprising an adhesive interface layer between the hole blocking layer and the adjacent photoge-

nerating layer to improve adhesion or to act as an electrical barrier layer, is disclosed, for example, in U.S. Pat. No. 4,780,385. Typical adhesive interface layers disclosed in U.S. Pat. No. 4,780,385 include film-forming polymers such as polyester, polyvinylbutyral, polyvinylpyrrolidone, polyurethane, polycarbonates polymethylmethacrylate, mixtures thereof, and the like. Specific polyester adhesive materials are disclosed, for example in U.S. Pat. No. 4,786,570 where linear saturated copolymers consisting of alternating monomer units of ethylene glycol and four randomly sequenced diacids and copolymers of diacids and diols where the diacid is selected from the group consisting of terephthalic acid, isophthalic acid, adipic acid, azelaic acid, and mixtures thereof and the diol is selected from the group consisting of ethylene glycol, 2,2-dimethyl propane diol and mixtures thereof. The entire disclosure of U.S. Pat. No. 4,786,570 is incorporated herein by reference.

An encouraging advance in electrophotographic imaging which has emerged in recent years is the successful fabrication of a flexible imaging member which exhibits excellent capacitive charging characteristic, outstanding photo-sensitivity, low electrical potential dark decay, and long term electrical cyclic stability. This imaging member employed in belt form usually comprises a substrate, a conductive layer, a solution coated hole blocking layer, a solution coated adhesive layer, a thin charge generating layer comprising a sublimation deposited perylene or phthalocyanine organic pigment or a dispersion of one of these pigments in a selected binder resin, a solution coated charge transport layer, a solution coated anti-curl layer, and an optional overcoating layer.

Multi-layered photoreceptors containing charge generating layers, comprising either vacuum sublimation deposited pure organic pigment or an organic pigment dispersion of perylene or phthalocyanine in a resin binder, have frequently been found to have undesirable characteristics such as forming charge deficient spots which are visible in the final hard copy print. Photoreceptors containing perylene pigments in the charge generating layers, particularly benzimidazole perylene dispersion charge generating layers, have a spectral sensitivity of up to 720 nanometers, are highly compatible with exposure systems utilizing visible laser diodes, exhibit low dark decay electrical characteristic and reduced background/residual voltages. These characteristics are superior to photoreceptor counterparts containing a trigonal selenium dispersion in the charge generating layer. Unfortunately, these multi-layered benzimidazole perylene photoreceptors have also been found to develop a serious charge deficient spots problem, particularly the dispersion of perylene pigment in the matrix of a bisphenol Z type polycarbonate film forming binder. The expression "charge deficient spots" as employed herein is defined as localized areas of dark decay that appear as toner deficient spots when using charged area development, e.g. appearance of small white spots having an average size of between about 0.2 and about 0.3 millimeter on a black toner background on an imaged hard copy. In discharged area development systems, the charge deficient spots appear in the output copies as small black toner spots on a white background. Moreover, multi-layered benzimidazole perylene photoreceptors have also been noted to yield low adhesion bond strength at the contacting surfaces between the charge generating layer and the adhesive interface layer, causing undesirable premature photoreceptor layer delamination during photoreceptor image cycling in copiers, duplicators and printers. In a customer service environment, premature photoreceptor layer delamination requires costly and frequent photoreceptor belt replacement by skilled technical representatives.

Typically, flexible photoreceptor belts are fabricated by depositing the various layers of photoactive coatings onto long webs which are thereafter cut into sheets. The opposite ends of each photoreceptor sheet are overlapped and ultrasonically welded together to form an imaging belt. In order to increase throughput during the web coating operation, the webs to be coated have a width of twice the width of a final belt. After coating, the web is slit lengthwise and thereafter transversely cut into predetermined length to form photoreceptor sheets of precise dimensions that are eventually welded into belts. When multi-layered photoreceptors containing perylene pigment dispersion in the charge generating layer are slit lengthwise during the belt fabrication process, it has been found that some of the photoreceptor delaminates and becomes unusable. In the fabricated belt form, photoreceptor layer delamination at the welded seam, due to stress concentration development at the double thickness overlap area during dynamic fatigue photoreceptor belt bending/flexing over the machine belt support rollers, diminishes the practical application value of the belt. All of the above deficiencies, implicated by the low layer adhesion bond strength, hinder slitting of a photoreceptor web through the charge generating layer without encountering edge delamination. Slitting is used to transversely cut webs into sheets for welding into belts and also to longitudinally slice double wide coated photoreceptor webs into multiple narrower charge generating layers.

In general, photoconductive pigment loadings of 80 percent by volume in a binder resin or a mixed resins binder are highly desirable in the photogenerating layer to provide excellent photosensitivity. However, these dispersions are highly unstable to extrusion coating conditions, resulting in numerous coating defects that generate a large number of unacceptable material that must be scrapped when using extrusion coating of a dispersion of pigment in organic solution of polymeric binder. More stable dispersions can be obtained by reducing the pigment loading to 30-40 percent by volume, but in most cases the resulting "diluted" photo-generating layer could not provide adequate photosensitivity. Also, the dispersions of higher pigment loadings generally provided a generator layer with poor to adequate adhesion to either the underlying ground plane or adhesive layer, or the overlying transport layer when polyvinylbutyral binders are utilized in the charge generating layer. Many of these organic dispersions are quite unstable with respect to pigment agglomeration, resulting in dispersion settling and the formation of dark streaks and spots of pigment during the coating process. Normally, the polymeric binders which produce the best (most stable, therefore most manufacturable) dispersion suffer from deficiencies either in xerographic or mechanical properties, while the least stable dispersions provided the best possible mechanical and xerographic properties. The best compromise of manufacturability and xerographic/mechanical performance is obtained by use of a photogenerating layer containing benzimidazole perylene pigment dispersed in a bisphenol Z type polycarbonate film forming binder. However, when a polyester adhesive layer is employed in a photoreceptor in combination with a photogenerating layer containing benzimidazole perylene pigment dispersed in a bisphenol A type or a bisphenol Z type polycarbonate film forming binder, poor adhesion between the charge generator layer and the adhesive layer can cause spontaneous photoreceptor delamination during certain slitting operations, during fabrication, or during extensive photoreceptor belt cycling over small diameter machine belt support rollers.

In addition, when a multilayered belt imaging member containing benzimidazole perylene pigment dispersed in the

bisphenol Z polycarbonate film forming binder in the charge generating layer is fabricated by ultrasonic welding the opposite ends of an imaging sheet together, delamination is encountered when attempts are made to grind away some of the weld splash material. Removal of the weld splash material is of particular important, because it allows the elimination of seams which form flaps during electrophotographic imaging and cleaning processes of belt function that causes the initiation of toner particles trapping and thereafter release them as unwanted dirts over the imaging belt surface to result in copy black spot print defects. Also, the inability to grind, buff, or polish a welded seam causes reduced cleaning blade life as well as seam interference with toner image ultrasonic transfer assist subsystems.

In U.S. Pat. No. 5,322,755 a layered photoconductive imaging member is disclosed comprising a supporting substrate, a photogenerator layer comprising perylene photoconductive pigments dispersed in a resin binder mixture comprising at least two polymers, and a charge transport layer. The resin binder can be, for example, a mixture of polyvinylcarbazole and polycarbonate homopolymer or a mixture of polyvinylcarbazole, polyvinylbutyral and polycarbonate homopolymer or a mixture of polyvinylcarbazole and polyvinylbutyral or a mixture of polyvinylcarbazole and a polyester. Although improvement in photosensitivity and adhesion are achieved, charge deficient spots print defects can still be a problem.

Thus, there is a continuing need for improved photoreceptors that exhibit freedom from charge deficient spots and are more resistant to layer delamination during slitting, grinding, buffing, polishing, and dynamic belt image cycling.

#### INFORMATION DISCLOSURE STATEMENT

U.S. Pat. No. 5,322,755 to Allen et al., issued on Jun. 21, 1994—A layered photoconductive imaging member is disclosed comprising a supporting substrate, a photogenerator layer comprising perylene photoconductive pigments dispersed in a resin binder mixture comprising at least two polymers, and a charge transport layer. The resin binder can be, for example, a mixture of polyvinylcarbazole and polycarbonate homopolymer or a mixture of polyvinylcarbazole, polyvinylbutyral and polycarbonate homopolymer or a mixture of polyvinylcarbazole and polyvinylbutyral or a mixture of polyvinylcarbazole and a polyester.

U.S. Pat. No. 5,418,100 to Yu, issued May 23, 1995—Discloses an electrophotographic imaging device fabrication method, in which the solvent used to coat charge transport layer is a solvent to which an underlying adhesive interface layer is substantially insensitive. The charge generating layer used for the imaging device is vacuum sublimation deposited benzimidazole perylene pigment and the adhesive interface layer may, for example, be formed of cross-linked film-forming polymers which are insoluble in a solvent used to apply the charge transport layer.

U.S. Pat. No. 4,925,760 to Baranyi et al., issued May 15, 1990—A layered photoresponsive imaging member is disclosed comprising a supporting substrate, a vacuum evaporated photogenerating layer comprised of certain pyranthrone pigments including tribromo-8,16-pyranthredione and trichloro-8,16-pyranthredione; and an aryl amine hole transport layer comprised of molecules of a certain designated formula dispersed in a resinous binder.

U.S. Pat. No. 4,780,385 to Wieloch et al., issued Oct. 25, 1988—An electrophotographic imaging member is dis-

closed having an imaging surface adapted to accept a negative electrical charge, the electrophotographic imaging member comprising a metal ground plane layer comprising zirconium, a hole blocking layer, a charge generation layer comprising photoconductive particles dispersed in a film forming resin binder, and a hole transport layer, the hole transport layer being substantially non-absorbing in the spectral region at which the charge generation layer generates and injects photogenerated holes but being capable of supporting the injection of photogenerated holes from the charge generation layer and transporting the holes through the charge transport layer.

U.S. Pat. No. 4,786,570 to Yu et al., issued Nov. 22, 1988—A flexible electrophotographic imaging member is disclosed which comprises a flexible substrate having an electrically conductive surface, a hole blocking layer comprising an aminosilane reaction product, an adhesive layer having a thickness between about 200 angstroms and about 900 angstroms consisting essentially of at least one copolyester resin having a specified formula derived from diacids selected from the group consisting of terephthalic acid, isophthalic acid, and mixtures thereof and a diol comprising ethylene glycol, the mole ratio of diacid to diol being 1:1, the number of repeating units equaling a number between about 175 and about 350 and having a  $T_g$  of between about 50° C. to about 80° C., the aminosilane also being a reaction product of the amino group of the silane with the —COOH and —OH end groups of the copolyester resin, a charge generation layer comprising a film forming polymeric component, and a diamine hole transport layer, the hole transport layer being substantially non-absorbing in the spectral region at which the charge generation layer generates and injects photogenerated holes but being capable of supporting the injection of photogenerated holes from the charge generation layer and transporting the holes through the charge transport layer. Processes for fabricating and using the flexible electrophotographic imaging member are also disclosed.

U.S. Pat. No. 5,019,473 to Nguyen et al., issued May 28, 1991—An electrophotographic recording element is disclosed having a layer comprising a photoconductive perylene pigment, as a charge generation material, that is sufficiently finely and uniformly dispersed in a polymeric binder to provide the element with excellent electrophotographic speed. The perylene pigments are perylene-3,4,9, 10-tetracarboxylic acid imide derivatives.

U.S. Pat. No. 4,587,189 to Hor et al., issued May 6, 1986—Disclosed is an improved layered photoresponsive imaging member comprised of a supporting substrate; a vacuum evaporated photogenerator layer comprised of a perylene pigment selected from the group consisting of a mixture of bisbenzimidazo(2,1-a-1',2'-b)anthra(2,1,9-def:6, 5,10 -d'e'f')diisoquinoline-6,11- dione, and bisbenzimidazo(2,1-a:2',1'a)anthra(2,1,9-def:6,5,10- d'e'f')diisoquinoline-10,21 -dione, and N,N'-diphenyl-3,4,9, 10-perylenebis(dicarboximide); and an aryl amine hole transport layer comprised of molecules of a specified formula dispersed in a resinous binder.

U.S. Pat. No. 4,588,667 to Jones et al., issued May 13, 1986—An electrophotographic imaging member is disclosed comprising a substrate, a ground plane layer comprising a titanium metal layer contiguous to the substrate, a charge blocking layer contiguous to the titanium layer, a charge generating binder layer and a charge transport layer. This photoreceptor may be prepared by providing a substrate in a vacuum zone, sputtering a layer of titanium metal on the substrate in the absence of oxygen to deposit a titanium

metal layer, applying a charge blocking layer, applying a charge generating binder layer and applying a charge transport layer. If desired, an adhesive layer may be interposed between the charge blocking layer and the photoconductive insulating layer.

U.S. Pat. No. 4,943,508 to Yu, issued Jul. 24, 1990—A process for fabricating an electrophotographic imaging member is disclosed which involves providing an electrically conductive layer, forming an aminosilane reaction product charge blocking layer on the electrically conductive layer, extruding a ribbon of a solution comprising an adhesive polymer dissolved in at least a first solvent on the electrically conductive layer to form a wet adhesive layer, drying the adhesive layer to form a dry continuous coating having a thickness between about 0.08 micrometer (800 angstroms) and about 0.3 micrometer (3,000 angstroms), applying to the dry continuous coating a mixture comprising charge generating particles dispersed in a solution of a binder polymer dissolved in at least a second solvent to form a wet generating layer, the binder polymer being miscible with the adhesive polymer, drying the wet generating layer to remove substantially all of the second solvent, and applying a charge transport layer, the adhesive polymer consisting essentially of a linear saturated copolyester reaction product of ethylene glycol and four diacids wherein the diol is ethylene glycol, the diacids are terephthalic acid, isophthalic acid, adipic acid and azelaic acid, the sole ratio of the terephthalic acid to the isophthalic acid to the adipic acid to the azelaic acid is between about 3.5 and about 4.5 for terephthalic acid; between about 3.5 and about 4.5 isophthalic acid; between about 0.5 and about 1.5 for adipic acid; between about 0.5 and about 1.5 for azelaic acid, the total moles of diacid being in a mole ratio of diacid to ethylene glycol in the copolyester of 1:1, and the  $T_g$  of the copolyester resin being between about 32° C. about 50° C.

U.S. Pat. No. 4,464,450 to Teuscher, issued Aug. 7, 1984—An electrostatographic imaging member is disclosed having two electrically operative layers including a charge transport layer and a charge generating layer, the electrically operative layers overlying a siloxane film coated on a metal oxide layer of a metal conductive anode, said siloxane film comprising a reaction product of a hydrolyzed silane having a specified general formula.

#### CROSS REFERENCE TO RELATED APPLICATIONS

This application is related to the following U.S. Patent Applications:

U.S patent application Ser. No. 08/587,120. (Attorney Docket No. D/94852), filed concurrently herewith in the names of Satchidanand Mishra et al., entitled "MULTILAYERED PHOTORECEPTEOR WITH ADHESIVE AND INTERMEDIATE LAYERS"—An electrophotographic imaging member is disclosed including a support substrate having an electrically conductive ground plane layer comprising a layer comprising zirconium over a layer comprising titanium a hole blocking layer, an adhesive layer comprising a polyester film forming resin, an intermediate layer in contact with the adhesive layer, the intermediate layer comprising a carbazole polymer, a charge generation layer comprising a perylene or a phthalocyanine, and a hole transport layer, said hole transport layer being substantially non-absorbing in the spectral region at which the charge generation layer generates and injects photogenerated holes but being capable of supporting the injection of photoge-

enerated holes from said charge generation layer and transporting said holes through said charge transport layer.

U.S. patent application Ser. No. 08/586,470 (Attorney Docket No. D/95064), filed concurrently herewith in the name of Robert C. U. Yu et al., entitled "PHOTORECEP-TOR-WHICH RESISTS CHARGE DEFICIENT SPOTS"—An electrophotographic imaging member comprising a support substrate having an electrically conductive ground plane layer comprising a layer comprising zirconium over a layer comprising titanium, a hole blocking layer, an adhesive layer comprising a thermoplastic polyurethane film forming resin, a charge generation layer comprising perylene or a phthalocyanine particles dispersed in a polycarbonate film forming binder, and a hole transport layer, said hole transport layer being substantially non-absorbing in the spectral region at which the charge generation layer generates and injects photogenerated holes but being capable of supporting the injection of photogenerated holes from said charge generation layer and transporting said holes through said charge transport layer.

U.S. patent application Ser. No. 08/586,469 (Attorney Docket No. D/95068), filed concurrently herewith in the name of Satchidanand Mishra et al., entitled "IMPROVED CHARGE GENERATION LAYER IN AN ELECTROPHOTOGRAPHIC IMAGING MEMBER"—An electrophotographic imaging member is disclosed comprising a support substrate having an electrically conductive ground plane layer comprising a layer comprising zirconium over a layer comprising titanium, a hole blocking layer, an adhesive layer comprising a polyester film forming resin, an intermediate layer in contact with the adhesive layer, the intermediate layer comprising a carbazole polymer, a charge generation layer comprising perylene or a phthalocyanine particles dispersed in a polymer binder blend of polycarbonate and carbazole polymer, and a hole transport layer, said hole transport layer being substantially non-absorbing in the spectral region at which the charge generation layer generates and injects photogenerated holes but being capable of supporting the injection of photogenerated holes from said charge generation layer and transporting said holes through said charge transport layer.

U.S. patent application Ser. No. 08/587,119 (Attorney Docket No. D/95065), filed concurrently herewith in the names of Satchidanand Mishra et al., entitled "ELECTROPHOTOGRAPHIC IMAGING MEMBER WITH IMPROVED CHARGE GENERATION LAYER"—An electrophotographic imaging member is disclosed including a support substrate having an electrically conductive ground plane layer comprising a layer comprising zirconium over a layer comprising titanium, a hole blocking layer, an adhesive layer comprising a copolyester resin, a charge generation layer comprising a perylene or a phthalocyanine particles dispersed in a film forming resin binder blend, said binder blend consisting essentially of a film forming polyvinyl butyral copolymer and a film forming copolyester, and a hole transport layer, said hole transport layer being substantially non-absorbing in the spectral region at which the charge generation layer generates and injects photogenerated holes but being capable of supporting the injection of photogenerated holes from said charge generation layer and transporting said holes through said charge transport layer.

U.S. patent application Ser. No. 08/587,118 (Attorney Docket No. D/93644), filed concurrently herewith in the name of Robert C. U. Yu, entitled "MULTILAYERED ELECTROPHOTOGRAPHIC IMAGING MEMBER WITH VAPOR DEPOSITED GENERATOR LAYER AND IMPROVED ADHESIVE LAYER"—An electrophoto-

graphic imaging member is disclosed comprising an electrophotographic imaging member comprising a substrate layer having an electrically conductive outer surface, an adhesive layer comprising a thermoplastic polyurethane film forming resin, a thin vapor deposited charge generating layer consisting essentially of a thin homogeneous vacuum sublimation deposited film of an organic photogenerating pigment, and a charge transport layer, the transport layer being substantially non-absorbing in the spectral region at which the charge generation layer generates and injects photogenerated holes but being capable of supporting the injection of photogenerated holes from the charge generation layer and transporting the holes through the charge transport layer.

#### SUMMARY OF THE INVENTION

It is, therefore, an object of the present invention to provide an improved photoreceptor member which overcomes the above-noted disadvantages.

It is yet another object of the present invention to provide an improved electrophotographic member having an intermediate layer which imparts to the member greater resistance to the formation of charge deficient spots during image cycling.

It is a further object of the present invention to provide a photoconductive imaging member which enables successful slitting a wide web lengthwise through a charge generation layer comprising benzimidazole perylene dispersed in a matrix of poly(4,4'-diphenyl-1,1'-cyclohexane carbonate).

It is still yet another object of the present invention to provide an improved electrophotographic member having an intermediate layer which renders greater adhesion bond strength with the charge generation layer

It is still another object of the present invention to provide an electrophotographic imaging member having welded seams that can be buffed or ground without causing layer delamination.

It is another object of the present invention to provide an electrophotographic imaging member which exhibits lower dark decay, reduced background and residual voltages, and improved cyclic stability, as well as having a photoresponse to a visible laser diode.

The foregoing objects and others are accomplished in accordance with this invention by providing an electrophotographic imaging member comprising a support substrate having a two layered electrically conductive ground plane layer comprising a layer comprising zirconium over a layer comprising titanium, a hole blocking layer, an adhesive layer comprising a polymer blend comprising a carbazole polymer and a thermoplastic resin selected from the group consisting of copolyester, polyarylate and polyurethane in contiguous contact with the hole blocking layer, a charge generation layer comprising perylene or a phthalocyanine pigment particles dispersed in a polycarbonate film forming binder in contiguous contact with the adhesive layer, and a hole transport layer, the hole transport layer being substantially non-absorbing in the spectral region at which the charge generation layer generates and injects photogenerated holes but being capable of supporting the injection of photogenerated holes from the charge generation layer and transporting the holes through the charge transport layer. This photoreceptor is utilized in an electrophotographic imaging process.

The substrate may be opaque or substantially transparent and may comprise numerous suitable materials having the required mechanical properties. Accordingly, this substrate

may comprise a layer of an electrically non-conductive or conductive material such as an inorganic or an organic composition. As electrically non-conducting materials there may be employed various thermoplastic and thermoset resins known for this purpose including polyesters, polycarbonates, polyamides, polyurethanes, and the like or metals such as aluminum, nickel, steel, stainless steel, titanium, chromium, copper, brass, tin, and the like. The substrate may have any suitable shape such as, for example, a flexible web, rigid cylinder, sheet and the like. Preferably, the substrate support is in the form of an endless flexible belt.

The thickness of a flexible substrate support depends on numerous factors, including economical considerations, and thus this layer for a flexible belt may be of substantial thickness, for example, over 200 micrometers, or of minimum thickness less than 50 micrometers, provided there are no adverse affects on the final photoconductive device. In one flexible belt embodiment, the thickness of this layer ranges from about 65 micrometers to about 150 micrometers, and preferably from about 75 micrometers to about 125 micrometers for optimum flexibility and minimum stretch when cycled around small diameter rollers, e.g. 12 millimeter diameter rollers.

The zirconium and/or titanium layer may be formed by any suitable coating technique, such as vacuum deposition. Typical vacuum depositing techniques include sputtering, magnetron sputtering, RF sputtering, and the like. Magnetron sputtering of zirconium or titanium onto a metallized substrate can be effected by a conventional type sputtering module under vacuum conditions in an inert atmosphere such as argon, neon, or nitrogen using a high purity zirconium or titanium target. The vacuum conditions are not particularly critical. In general, a continuous zirconium or titanium film can be attained on a suitable substrate, e.g. a polyester web substrate such as Mylar available from E. I. du Pont de Nemours & Co. with magnetron sputtering. It should be understood that vacuum deposition conditions may all be varied in order to obtain the desired zirconium or titanium thickness. Typical techniques for forming the zirconium and titanium layers are described in U.S. Pat Nos. 4,780,385 and 4,588,667, the entire disclosures of which are incorporated herein in their entirety.

The conductive layer comprises a plurality of metal layers with the outermost metal layer (i.e. the layer closest to the charge blocking layer) comprising at least 50 percent by weight of zirconium. At least 70 percent by weight of zirconium is preferred in the outermost metal layer for even better results. The multiple layers may, for example, all be vacuum deposited or a thin layer can be vacuum deposited over a thick layer prepared by a different techniques such as by casting. Thus, as an illustration, a zirconium metal layer may be formed in a separate apparatus than that used for previously depositing a titanium metal layer or multiple layers can be deposited in the same apparatus with suitable partitions between the chamber utilized for depositing the titanium layer and the chamber utilized for depositing zirconium layer. The titanium layer may be deposited immediately prior to the deposition of the zirconium metal layer. Generally, for rear erase exposure, a conductive layer light transparency of at least about 15 percent is desirable. The combined thickness of the two layered conductive layer should be between about 120 and about 300 angstroms. A typical zirconium/titanium dual conductive layer has a total combined thickness of about 200 angstroms. Although thicker layers may be utilized, economic and transparency considerations may affect the thickness selected.

Regardless of the technique employed to form the zirconium and/or titanium layer, a thin layer of zirconium or

titanium oxide forms on the outer surface of the metal upon exposure to air. Thus, when other layers overlying the zirconium layer are characterized as "contiguous" layers, it is intended that these overlying contiguous layers may, in fact, contact a thin zirconium or titanium oxide layer that has formed on the outer surface of the metal layer. If the zirconium and/or titanium layer is sufficiently thick to be self supporting, no additional underlying member is needed and the zirconium and/or titanium layer may function as both a substrate and a conductive ground plane layer. Ground planes comprising zirconium tend to continuously oxidize during xerographic cycling due to anodizing caused by the passage of electric currents, and the presence of this oxide layer tends to decrease the level of charge deficient spots with xerographic cycling. Generally, a zirconium layer thickness of at least about 100 angstroms is desirable to maintain optimum resistance to charge deficient spots during xerographic cycling. A typical electrical conductivity for conductive layers for electrophotographic imaging members in slow speed copiers is about  $10^2$  to  $10^3$  ohms/square.

After deposition of the zirconium an/or titanium metal layer, a hole blocking layer is applied thereto. Generally, electron blocking layers for positively charged photoreceptors allow the photogenerated holes in the charge generating layer at the top of the photoreceptor to migrate toward the charge (hole) transport layer below and reach the bottom conductive layer during the electrophotographic imaging processes. Thus, an electron blocking layer is normally not expected to block holes in positively charged photoreceptors such as photoreceptors coated with charge a generating layer over a charge (hole) transport layer. For negatively charged photoreceptors, any suitable hole blocking layer capable of forming an electronic barrier to holes between the adjacent photoconductive layer and the underlying zirconium and/or titanium layer may be utilized. A hole blocking layer may comprise any suitable material. Typical hole blocking layers utilized for the negatively charged photoreceptors may include, for example, Luckamide, hydroxy alkyl methacrylates, nylons, gelatin, hydroxyl alkyl cellulose, organopolyporphazines, organosilanes, organotitanates, organozirconates, silicon oxides, zirconium oxides, and the like. Preferably, the hole blocking layer comprises nitrogen containing siloxanes. Typical nitrogen containing siloxanes are prepared from coating solutions containing a hydrolyzed silane. Typical hydrolyzable silanes include 3-aminopropyl triethoxy silane, (N,N'-dimethyl 3-amino)propyl triethoxysilane, N,N-dimethylamino phenyl triethoxy silane, N-phenyl aminopropyl trimethoxy silane, trimethoxy silylpropyl diethylene triamine and mixtures thereof.

During hydrolysis of the amino silanes described above, the alkoxy groups are replaced with hydroxyl group. An especially preferred blocking layer comprises a reaction product between a hydrolyzed silane and the zirconium and/or titanium oxide layer which inherently forms on the surface of the metal layer when exposed to air after deposition. This combination reduces spots at time 0 and provides electrical stability at low RH. The imaging member is prepared by depositing on the zirconium and/or titanium oxide layer of a coating of an aqueous solution of the hydrolyzed silane at a pH between about 4 and about 10, drying the reaction product layer to form a siloxane film and applying electrically operative layers, such as a photogenerator layer and a hole transport layer, to the siloxane film.

The blocking layer may be applied by any suitable conventional technique such as spraying, dip coating, draw bar coating, gravure coating, silk screening, air knife coating, reverse roll coating, vacuum deposition, chemical treat-

ment and the like. For convenience in obtaining thin layers, the blocking layers are preferably applied in the form of a dilute solution, with the solvent being removed after deposition of the coating by conventional techniques such as by vacuum, heating and the like. This siloxane coating is described in U.S. Pat. No. 4,464,450 to L. A. Teuscher, the disclosure of thereof being incorporated herein in its entirety. After drying, the siloxane reaction product film formed from the hydrolyzed silane contains larger molecules. The reaction product of the hydrolyzed silane may be linear, partially crosslinked, a dimer, a trimer, and the like.

The siloxane blocking layer should be continuous and have a thickness of less than about 0.5 micrometer because greater thicknesses may lead to undesirably high residual voltage. A blocking layer of between about 0.005 micrometer and about 0.3 micrometer (50 Angstroms-3000 Angstroms) is preferred because charge neutralization after the exposure step is facilitated and optimum electrical performance is achieved. A thickness of between about 0.03 micrometer and about 0.06 micrometer is preferred for zirconium and/or titanium oxide layers for optimum electrical behavior and reduced charge deficient spot occurrence and growth.

The adhesive layer of this invention is applied to the charge blocking layer. The adhesive layer comprises any suitable film forming copolyester resin and polyvinylcarbazole to form a polymer blend adhesive interface layer. A preferred copolyester resin is a linear saturated copolyester reaction product of four diacids and ethylene glycol. The molecular structure of this linear saturated copolyester having the following structural formula:



where n is the degree of polymerization which is between about 170 and about 370. The mole ratio of diacid of ethylene glycol in the copolyester is 1:1. The diacids are terephthalic acid, isophthalic acid, adipic acid and azelaic acid. The mole ratio of terephthalic acid to isophthalic acid to adipic acid to azelaic acid is 4:4:1:1. A representative linear saturated copolyester adhesion promoter of this structure is commercially available as Mor-Ester 49,000 (available from Morton International Inc., previously available from dupont de Nemours & Co.). The Mor-Ester 49,000 is a linear saturated copolyester which consists of alternating monomer units of ethylene glycol and four randomly sequenced diacids in the above indicated ratio and n in the structural formula has a value which gives a weight average molecular weight of about 70,000. This linear saturated copolyester has a  $T_g$  of about 32° C. Another preferred representative polyester resin is a copolyester resin having the above structural formula is one where the diacid is selected from the group consisting of terephthalic acid, isophthalic acid, and mixtures thereof; the diol is selected from the group consisting of ethylene glycol, 2,2-dimethyl propane and mixtures thereof; the ratio of diacid to diol is 1:1; n is a number between about 175 and about 350 and the  $T_g$  of the copolyester resin is between about 50° C. about 80° C. Typical polyester resins having the above structure are commercially available and include, for example, Vitel PE-100, Vitel PE-200, Vitel PE-200D, and Vitel PE-222, all available from Goodyear Tire and Rubber Co. More specifically, Vitel PE-100 polyester resin is a linear saturated copolyester of two diacids and ethylene glycol where the ratio of diacid to ethylene glycol in this copolyester is 1:1. The diacids are terephthalic acid and isophthalic acid. The

ratio of terephthalic acid to isophthalic acid is 3:2. The molecular structures of these acids and ethylene glycol are present above. The Vitel PE-100 linear saturated copolyester consists of alternating monomer units of ethylene glycol and two randomly sequenced diacids in the above indicated ratio and has a weight average molecular weight of about 50,000 and a  $T_g$  of about 71° C. This copolyester has the following formula:

$$y(t) = \frac{1}{2\tau_0} \sum_{\tau=-\tau_0}^{\tau_0} W(\tau) x(t+\tau)$$

wherein

said diacid is selected from the group consisting of terephthalic acid, isophthalic acid, and mixtures thereof,

said diol comprises ethylene glycol and 2,2-dimethyl propane diol,

said mole ratio of diacid to diol is 1:1, said mole ratio of terephthalic acid to isophthalic acid is 1.2:1, said mole ratio of ethylene glycol to 2,2-dimethyl propane diol is 1.33:1,

n is a number between about 160 and about 330, and the  $T_g$  of said copolyester resin is between about 50° C. and about 80° C.

Another polyester resin, represented by the above formula, is Vitel PE-200 available from Goodyear Tire & Rubber Co. This polyester resin is a linear saturated copolyester of two diacids and two diols where the ratio of diacid to diol in the copolyester is 1:1. The diacids are terephthalic acid and isophthalic acid. The ratio of terephthalic acid to isophthalic acid is 1.2:1. The two diols are ethylene glycol and 2,2-dimethyl propane diol. The ratio of ethylene glycol to dimethyl propane diol is 1.33:1. The Goodyear PE-200 linear saturated copolyester consists of randomly alternating monomer units of the two diacids and the two diols in the above indicated ratio and has a weight average molecular weight of about 45,000 and a  $T_g$  of about 67° C.

The diacids from which the polyester resins of this invention are derived are terephthalic acid, isophthalic acid, adipic acid and/or azelaic acid acids only. Any suitable diol may be used to synthesize the polyester resins employed in the adhesive layer of this invention typical diols includem, for example, ethylene glycol, 2,2-dimethyl propane diol, butane diol, pentane diol, hexane diol, and the like.

The adhesive interface layer of this invention may also comprise a carbazole polymer binder or a binder consisting of a mixture of carbazole polymers having the molecular strutures (A), (B), (C), and (D) as shown in the following:





wherein n, the degree of polymerization, is number of 20  
between about 800 and about 6,000.

The above structure (A), polyvinylcarbazole, is of particular interest because is readily commercially available from BASF Corporation. The polyvinyl carbazole has a weight average weight between about 750,000 and about 1,000,000. Satisfactory results are achieved when the weight ratio of polyvinylcarbazole to linear copolyester in the adhesive layer of this invention is between about 90:5 and about 50:50. For optimum adhesion a ration of about 75:25 ratio of polyvinylcarbazole to linear copolyester is preferred. Preferably the dried adhesive layer comprises between about 80 percent and about 95 percent of the polyvinylcarbazole and linear copolyester combination, based on the total weight of the dried adhesive layer.

Optionally, the adhesive interface layer of this invention may contain an arylamine. Typical arylamines have the general formula:



wherein R<sub>1</sub> and R<sub>2</sub> are an aromatic group selected from the group consisting of a substituted or unsubstituted phenyl group, naphthyl group, and polyphenyl group and R<sub>3</sub> is selected from the group consisting of a substituted or unsubstituted aryl group, alkyl group having from 1 to 18 carbon atoms and cycloaliphatic compounds having from 3 to 18 carbon atoms. The substituents should be free form electron withdrawing groups such as NO<sub>2</sub> groups, CN groups, and the like. Examples of charge transporting aromatic amines represented by the structural formula above include triphenylmethane, bis(4-diethylamine-2-methylphenyl)phenylmethane; 4'-4"-bis(diethylamino)-2',2"-dimethyl-triphenylmethane, N,N'-bis(alkylphenyl)-[1,1'-biphenyl]-4,4'-diamine wherein the alkyl is, for example, methyl, ethyl, propyl, n-butyl, etc., N,N'-diphenyl-N,N'-bis(chlorophenyl)-[1,1'-biphenyl]-4,4'-diamine, N,N'-diphenyl-N,N'-bis(3"-methylphenyl)-(1,1'-biphenyl)-4,4'-diamine, and the like. Generally, the adhesive layer of this invention can contain up to about 10 percent by weight of the arylamine, based on the total weight of the dried adhesive layer. Addition of an arylamine to the adhesive layer stabilizes the thickness of the adhesive layer by preventing swelling due to diffusion of arylamine from overlying layers which is difficult to control.

Any suitable solvent may be used to form an adhesive layer coating solution. Typical solvents include tetrahydro-

**14**

furan, toluene, hexane, cyclohexane, cyclohexanone, methylene chloride, 1,1,2-trichloroethane, monochlorobenzene, and the like, and mixtures thereof. Any suitable technique may be utilized to apply the adhesive layer coating. Typical coating techniques include extrusion coating, gravure coating, spray coating, wire wound bar coating, and the like. The adhesive layer comprising the polyester resin, polyvinylcarbazole and optional arylamine is applied directly to the charge blocking layer. Thus, the adhesive layer of this invention is in direct contiguous contact with both the underlying charge blocking layer and the overlying charge generating layer to enhance adhesion bonding and to effect ground plane hole injection suppression. Drying of the deposited coating may be effected by any suitable conventional process such as oven drying, infra red radiation drying, air drying and the like. The adhesive layer of this invention should be continuous. Satisfactory results are achieved when the adhesive layer has a thickness between about 0.03 micrometer and about 2 micrometers after drying. Preferably, the dried thickness is between about 0.05 micrometer and about 1 micrometer. At thickness of less than about 0.03 micrometer, the adhesion between the charge generating layer and the blocking layer is poor and delamination can occur when the photoreceptor belt is transported over small diameter supports such as rollers and curved skid plates. When the thickness of the adhesive layer of this invention is greater than about 2 micrometers, excessive residual charge buildup is observed during extended cycling.

Surprisingly, the adhesive interface layers of this invention comprising polyester, polyvinylcarbazole and an optional arylamine provides markedly superior electrical and adhesive properties when it is employed between an adhesive layer and a charge generation layer. Moreover, when used in contact with a charge generating layer comprising benzimidazole perylene dispersed in a film forming resin binder of poly(4,4'-diphenyl-1,1'-cyclohexane carbonate), slitting of a production imaging member web can be successfully carried-out without exhibition of spontaneous edge delamination. In addition, grinding at the ultrasonic welded seam to reduce the imaging member belt seam thickness is possible without causing seam overlap cracking/delamination problem.

Alternatively, the adhesive interface layer of this invention may also comprises a polymer blend of polyarylate (ARDEL D-100, available from Amoco Performance Products, Inc.) and a carbazole polymer, having between about 95:5 and 50:50 weight ratio of carbazole polymer to polyarylate. Polyarylates have the following repeating structural units:



Still another adhesive interface layer for the photoreceptor of this invention comprises a polymer blend of a thermoplastic polyurethane and a carbazole polymer, having between about 90:10 and 10:90 weight ratio of carbazole polymer to thermoplastic polyurethane, is also within the scope of the present invention. A preferred polyurethane has the following structural formula:



5

wherein

R is diphenyl substituted methylene group or dicyclohexyl substituted methylene group,

R' is a straight alkyl chain hydrocarbon containing 10 between 2 and 6 carbon atoms, and

J is, the degree of polymerization, between 90 and 500.

The charge generating layer of the photoreceptor of this invention comprises a vacuum sublimation deposited perylene or phthalocyanine organic pigment. The charge generating layer of the photoreceptor of this invention may also comprise an organic pigment, either perylene or phthalocyanine dispersion in a film forming resin. It is preferably that the perylene pigment is benzimidazole perylene which is also referred to as bis(benzimidazole). This pigment exists in the cis and trans forms. The cis form is also called bis-benzimidazo(2,1-a'1',1'-b)anthra(2,1,9-def:6,5,10-d'e'f)disoquinoline-6,11-dione. The trans form is also called bisbenzimidazo(2,1-a'1',1'-b)anthra(2,1,9-def:6,5,10-d'e'f)disoquinoline-10,21-dione. This pigment may be prepared by reacting perylene 3,4,9,10-tetracarboxylic acid dianhydride with 1,2-phenylene as illustrated in the following equation:



wherein "S" in the formula represents saturation. Preferably, the film forming polycarbonate binder for the charge generating layer has a molecular weight between about 20,000 and about 80,000. Satisfactory results may be achieved when the dried charge generating layer contains between about 20 percent and about 90 percent by volume benzimidazole perylene dispersed in poly(4,4'-diphenyl-1,1'-cyclohexane carbonate) based on the total volume of the dried charge generating layer. Preferably, the perylene pigment is present in an amount between about 30 percent and about 80 percent by volume. Optimum results are achieved with an amount between about 35 percent and about 45 percent by volume. Poly(4,4'-diphenyl-1,1'-cyclohexane carbonate) allow a reduction in perylene pigment loading without an extreme loss in photosensitivity.

Preferably, the charge generating layer also comprises up to about 60 percent by weight polyvinylcarbazole based on the total weight of the dried charge generating layer. Preferably, the polyvinylcarbazole concentration is between about 50 percent and about 5 percent by weight. Optimum results are achieved with a polyvinylcarbazole concentration of between about 30 percent and about 10 percent by weight. When the concentration of polyvinylcarbazole is greater than about 60 percent by weight based on the total weight of the charge generating layer, poor polymer blending occurs which impacts both photoelectrical and mechanical function of the imaging member.

Any suitable solvent may be utilized to dissolve the polycarbonate binder. Typical solvents include tetrahydrofuran, toluene, methylene chloride, and the like. Tetrahydrofuran is preferred because it has no discernible adverse effects on xerography and has an optimum boiling point to allow adequate drying of the generator layer during a typical slot coating process. Coating dispersions for charge generating layer may be formed by any suitable technique using, for example, attritors, ball mills, Dymomills, paint shakers, homogenizers, microfluidizers, and the like.

Any suitable coating technique may be used to apply coatings. Typical coating techniques include slot coating, gravure coating, roll coating, spray coating, spring wound bar coating, dip coating, draw bar coating, reverse roll coating, and the like.

Any suitable drying technique may be utilized to solidify and dry the deposited coatings. Typical drying techniques include oven drying, forced air drying, infrared radiation drying, and the like.

Satisfactory results may be achieved with a dry charge generating layer thickness between about 0.3 micrometer and about 3 micrometers. Preferably, the charge generating layer has a dried thickness of between about 1.1 micrometers and about 2 micrometers. The photogenerating layer thickness is related to binder content. Thicknesses outside these ranges can be selected providing the objectives of the present invention are achieved.

Any suitable charge transport layer may be utilized. The active charge transport layer may comprise any suitable transparent organic polymer of non-polymeric material capable of supporting the injection of photogenerated holes and electrons from the charge generating layer and allowing the transport of these holes or electrons through the organic layer to selectively discharge the surface charge. The charge transport layer in conjunction with the generation layer in the instant invention is a material which is an insulator to the extent that an electrostatic charge placed on the transport layer is not conducted in the absence of illumination. Thus, the active charge transport layer is a substantially non-photoconductive material which supports the injection of photogenerated holes from the generation layer.

An especially preferred transport layer employed in one of the two electrically operative layers in the multilayer photoconductor of this invention comprises from about 25 to about 75 percent by weight of at least one charge transporting aromatic amine compound, and about 75 to about 25 percent by weight of a polymeric film forming resin in which the aromatic amine is soluble. A dried charge transport layer containing between about 40 percent and about 50 percent by weight of the small molecule charge transport molecule based on the total weight of the dried charge transport layer is preferred.

The charge transport layer forming mixture preferably comprises an aromatic amine compound. Typical aromatic amine compounds include triphenyl amines, bis and poly triarylamines, bis arylamine ethers, bis alkylarylamines and the like.

Examples of charge transporting aromatic amines for charge transport layers capable of supporting the injection of photogenerated holes of a charge generating layer and transporting the holes through the charge transport layer include, for example, triphenylmethane, bis(4-diethylamino-2-methylphenyl)phenylmethane; 4'-4"-bis(diethylamino)-2', 2"-dimethyltriphenylmethane, N,N'-bis(alkylphenyl)-[1,1'-biphenyl]-4,4'-diamine wherein the alkyl is, for example, methyl, ethyl, propyl, n-butyl, etc., N,N'-diphenyl-N,N'-bis(chlorophenyl)-[1,1'-biphenyl]-4,4'-diamine, N,N'-diphenyl-N,N'-bis(3"-methylphenyl)-(1,1'-biphenyl)-4,4'-diamine, and the like dispersed in an inactive resin binder.

Any suitable inactive resin binder soluble in methylene chloride or other suitable solvent may be employed in the process of this invention. Typical inactive resin binders soluble in methylene chloride include polycarbonate resin, polyvinylcarbazole, polyester, polyarylate, polyacrylate, polyether, polysulfone, and the like. Molecular weights can vary from about 20,000 to about 1,500,000.

The preferred electrically inactive resin materials are polycarbonate resins have a molecular weight from about 20,000 to about 120,000, more preferably from about 50,000 to about 100,000. The materials most preferred as the electrically inactive resin material is poly(4,4'-dipropylidene-diphenylene carbonate) with a molecular weight of from about 35,000 to about 40,000, available as Lexan 145 from General Electric Company; poly(4,4'-isopropylidene-diphenylene carbonate) with a molecular weight of from about 40,000 to about 45,000, available as Lexan 141 from the General Electric Company; a polycarbonate resin having a molecular weight of from about 50,000 to about 100,000, available as Makrolon from Farbenfabriken Bayer A. G. and a polycarbonate resin having a molecular weight of from about 20,000 to about 50,000 available as Merlon from Mobay Chemical Company.

Examples of photosensitive members having at least two electrically operative layers include the charge generator layer and diamine containing transport layer members disclosed in U.S. Pat. Nos. 4,265,990, 4,233,384, 4,306,008, 4,299,897 and 4,439,507. The disclosures of these patents are incorporated herein in their entirety.

Any suitable and conventional technique may be utilized to mix and thereafter apply the charge transport layer coating mixture to the charge generating layer. Typical application techniques include spraying, dip coating, roll coating, wire wound rod coating, and the like. Drying of the deposited coating may be effected by any suitable conventional technique such as oven drying, infra red radiation drying, air drying and the like. Generally, the thickness of the transport layer is between about 5 micrometers to about 100 micrometers, but thicknesses outside this range can also be used. A

dried thickness of between about 18 micrometers and about 35 micrometers is preferred with optimum results being achieved with a thickness between about 24 micrometers and about 29 micrometers.

Preferably, the charge transport layer comprises an arylamine small molecule dissolved or molecularly dispersed in a polycarbonate.

Other layers such as conventional ground strips comprising, for example, conductive particles disposed in a film forming binder may be applied to one edge of the photoreceptor in contact with the zirconium and/or titanium layer, blocking layer, adhesive layer or charge generating layer.

Optionally, an overcoat layer may also be utilized to improve resistance to abrasion. In some cases a back coating may be applied to the side opposite the photoreceptor to provide flatness and/or abrasion resistance. These overcoating and backcoating layers may comprise organic polymers or inorganic polymers that are electrically insulating or slightly semi-conductive.

The invention will now be described in detail with respect to the specific preferred embodiments thereof, it being understood that these examples are intended to be illustrative only and that the invention is not intended to be limited to the materials, conditions, process parameters and the like recited herein. All parts and percentages are by weight unless otherwise indicated.

#### COMPARATIVE EXAMPLE I

A photoconductive imaging member was prepared by providing a web of titanium and zirconium coated polyester (Melinex, available from ICI Americas Inc.) substrate having a thickness of 3 mils, and applying thereto, with a gravure applicator, a solution containing 50 grams 3-aminopropyltriethoxysilane, 15 grams acetic acid, 684.8 grams of 200 proof denatured alcohol and 200 grams heptane. This layer was then dried for about 5 minutes at 135° C. in the forced air drier of the coater. The resulting blocking layer had a dry thickness of 500 Angstroms.

An adhesive interface layer was then prepared by applying a wet coating over the blocking layer, using a gravure applicator, containing 3.5 percent by weight based on the total weight of the solution of copolyester adhesive (Mor-Ester 49,000, available from Morton International, Inc., previously available from E. I. du Pont de Nemours & Co.) in a 70:30 volume ratio mixture of tetrahydrofuran/cyclohexanone. The adhesive interface layer was then dried for about 5 minutes at 135° C. in the forced air drier of the coater. The resulting adhesive interface layer had a dry thickness of 620 Angstroms.

A 9 inch×12 inch sample was then cut from the web, and the adhesive interface layer was thereafter coated with a photogenerating layer (CGL) containing 40 percent by volume benzimidazole perylene and 60 percent by volume poly(4,4'-diphenyl-1,1'-cyclohexane carbonate). This photogenerating layer was prepared by introducing 0.3 grams of poly(4,4'-diphenyl-1,1'-cyclohexane carbonate) PCZ-200, available from Mitsubishi Gas Chem. and 48 ml of tetrahydrofuran into a 4 oz. amber bottle. To this solution was added 1.6 gram of benzimidazole perylene and 300 grams of 1/8 inch diameter stainless steel shot. This mixture was then placed on a ball mill for 96 hours. 10 grams of the resulting dispersion was added to a solution containing 0.547 grams of poly(4,4'-diphenyl-1,1'-cyclohexane carbonate) PCZ-200 and 6.14 grams of tetrahydrofuran. The resulting slurry was thereafter applied to the adhesive interface with a 1/2-mil gap Bird applicator to form a layer having a wet thickness of 0.5

mil. The layer was dried at 135° C. for 5 minutes in a forced air oven to form a dry thickness photogenerating layer having a thickness of about 1.2 micrometers.

This photogenerator layer was overcoated with a charge transport layer. The charge transport layer was prepared by introducing into an amber glass bottle in a weight ratio of a hole transporting molecule of 1:1 N,N'-diphenyl-N,N'-bis(3-methylphenyl)-1,1'-biphenyl-4,4'-diamine and Makrolon 5705, a polycarbonate resin having a molecular weight of from about 50,000 to 100,000 commercially available from Farbenfabriken Bayer A. G. The resulting mixture was dissolved in methylene chloride to form a solution containing 15 percent by weight solids. This solution was applied on the photogenerator layer using a 3-mil gap Bird applicator to form a coating which upon drying had a thickness of 24 microns. During this coating process the humidity was equal to or less than 15 percent. The photoreceptor device containing all of the above layers was annealed at 135° C. in a forced air oven for 5 minutes and thereafter cooled to ambient room temperature. After application of the charge transport layer coating, the imaging member spontaneous curled upwardly. An anti-curl coating was needed to impart the desired flatness to the imaging member. The anti-curl coating solution was prepared in a glass bottle by dissolving 8.82 grams polycarbonate (Makrolon 5705, available from Bayer AG) and 0.09 grams copolyester adhesion promoter (Vitel PE-100, available from Goodyear Tire and Rubber Company) in 90.07 grams methylene chloride. The glass bottle was then covered tightly and placed on a roll mill for about 24 hours until total dissolution of the polycarbonate and the copolyester is achieved. The anti-curl coating solution thus obtained was applied to the rear surface of the supporting substrate (the side opposite to the imaging layers) by hand coating using a 3 mil gap Bird applicator. The coated wet film was dried at 135° C. in an air circulation oven for about 5 minutes to produce a dry, 14 micrometer thick anti-curl layer and provide the desired imaging member flatness. The resulting photoconductive imaging member was used to serve as a control.

#### EXAMPLE II

A photocductive imaging member was prepared as described in Comparative Example I, except that the 49000 adhesive interface layer was substituted by an invention adhesive interface layer containing a 0.1 micrometer thick dried-coating of polyvinylcarbazole (available from BASF Corporation) and linear copolyester Mor-Ester 49,000 (available from Morton International Inc.) in a weight ratio of 95:5. This coating was applied with a 1/5-mil gap Bird applicator, using a 1 percent weight solid of 95 polyvinylcarbazole:5 Mor-Ester 49,000 weight ratio dissolved in tetrahydrofuran.

#### EXAMPLE III

A photocductive imaging member was prepared as described in Example II, except that the invention adhesive interface layer containing a 0.1 micrometer thick dried-coating of polyvinylcarbazole and linear copolyester Mor-Ester 49,000 in a weight ratio of 90:10.

#### EXAMPLE IV

A photocductive imaging member was prepared as described in Example II, except that the invention adhesive interface layer containing a 0.1 micrometer thick dried-coating of polyvinylcarbazole and linear copolyester Mor-

Ester 49,000 in a weight ratio of 85:15.

#### EXAMPLE V

A photocductive imaging member was prepared as described in Example II, except that the invention adhesive interface layer containing a 0.1 micrometer thick dried-coating of polyvinylcarbazole and linear copolyester Mor-Ester 49,000 in a weight ratio of 75:25.

#### EXAMPLE VI

A photocductive imaging member was prepared as described in Example II, except that the invention adhesive interface layer containing a 0.1 micrometer thick dried-coating of polyvinylcarbazole and linear copolyester Mor-Ester 49,000 in a weight ratio of 50:50.

#### EXAMPLE VI

A photocductive imaging member was prepared as described in Example II, except that the invention adhesive interface layer containing a 0.1 micrometer thick dried-coating of polyvinylcarbazole and linear copolyester Mor-Ester 49,000 in a weight ratio of 50:50. The invention adhesive interface layer also contained 10 weight percent of arylamine N,N'-diphenyl-N,N'-bis(3-methylphenyl)-1,1'-bi-phenyl-4,4'-diamine based on the total weight of the adhesive interface layer.

#### EXAMPLE VIII

A photocductive imaging member was prepared as described in Example II, except that the invention adhesive interface layer containing a 0.1 micrometer thick dried-coating of polyvinylcarbazole and polyarylate (ARDEL D-100, available from Amoco Performance Products, Inc.) in a weight ratio of 25:75.

#### EXAMPLE IX

A photocductive imaging member was prepared as described in Example II, except that the invention adhesive interface layer containing a 0.1 micrometer thick dried-coating of polyvinylcarbazole and polyarylate in a weight ratio of 50:50.

#### EXAMPLE X

A photocductive imaging member was prepared as described in Example II, except that the invention adhesive interface layer containing a 0.1 micrometer thick dried-coating of polyvinylcarbazole and thermoplastic polyether type polyurethane (Elastollan 1180A, available from BASF Corporation.) in a weight ratio of 20:80.

#### EXAMPLE XI

A photocductive imaging member was prepared as described in Example II, except that the invention adhesive interface layer containing a 0.1 micrometer thick dried-coating of polyvinylcarbazole and thermoplastic polyether-type polyurethane in a weight ratio of 50:50.

#### EXAMPLE XII

A photocductive imaging member was prepared as described in Example II, except that the invention adhesive interface layer containing a 0.1 micrometer thick dried-coating of polyvinylcarbazole and thermoplastic polyether-type polyurethane in a weight ratio of 80:20.

#### EXAMPLE XIII

The electrical properties of photocductive imaging members of Examples I through XII were evaluated with a xerographic testing scanner comprising a cylindrical aluminum drum having a diameter of 24.26 cm (9.55 inches). The test samples were taped onto the drum. When rotated, the drum carrying the samples produced a constant surface speed of 76.3 cm (30 inches) per second. A direct current pin corotron, exposure light, erase light, and five electrometer probes were mounted around the periphery of the mounted photoreceptor samples. The sample charging time was 33 milliseconds. Both expose and erase lights were broad band white light (400-700 nm) outputs, each supplied by a 300 watt output Xenon arc lamp. The relative locations of the probes and lights are indicated in Table A below:

TABLE A

| ELEMENT | ANGLE<br>(Degrees) | POSITION<br>(mm) | DISTANCE<br>FROM<br>PHOTORECEPTOR<br>(mm) |
|---------|--------------------|------------------|-------------------------------------------|
| Charge  | 0.0                | 0.0              | 18 (Pins)<br>12 (Shield)                  |
| Probe 1 | 22.50              | 47.9             | 3.17                                      |
| Expose  | 56.25              | 118.8            | N.A.                                      |
| Probe 2 | 78.75              | 166.8            | 3.17                                      |
| Probe 3 | 168.75             | 356.0            | 3.17                                      |
| Probe 4 | 236.25             | 489.0            | 3.17                                      |
| Erase   | 258.75             | 548.0            | 125.00                                    |
| Probe 5 | 303.75             | 642.9            | 3.17                                      |

The test samples were first rested in the dark for at least 60 minutes to ensure achievement of equilibrium with the testing conditions at 40 percent relative humidity and 21° C. Each sample was then negatively charged in the dark to a development potential of about 900 volts. The charge acceptance of each sample and its residual potential after discharge by front erase exposure to 400 ergs/cm<sup>2</sup> were recorded. The test procedure was repeated to determine the photo induced discharge characteristic (PIDC) of each sample by different light energies of up to 20 ergs/cm<sup>2</sup>.

The imaging member of Examples I to XII were again tested in a motionless scanner using a Differential Increase In Dark Decay (DIDD) measurement technique for charge deficient spot (microdefect) levels. The test involved the following steps:

- providing at least a first electrophotographic imaging member having a known differential increase in dark decay value, the imaging member comprising an electrically conductive layer and at least one photoconductive layer,
- repeatedly subjecting the at least one electrophotographic imaging member to cycles comprising electrostatic charging and light discharging steps,
- measuring dark decay of the at least one photoconductive layer during cycling until the amount of dark decay reaches a crest value,
- establishing with the crest value a first reference datum for dark decay crest value at an initial applied field between about 24 volts/micrometer and about 40 volts/micrometer,
- establishing with the crest value a second reference datum for dark decay crest value at a final applied field between about 64 volts/micrometer and about 80 volts/micrometer,
- determining the differential increase in dark decay between the first reference datum and the second ref-

erence datum for the first electrophotographic imaging member to establish a known differential increase in dark decay value,

- (g) repeatedly subjecting a virgin electrophotographic imaging member to aforementioned cycles comprising electrostatic charging and light discharging steps until the amount of dark decay reaches a crest value for the virgin which remains substantially constant during further cycling,
- (h) establishing with the crest value for the virgin electrophotographic imaging member a third reference datum for dark decay crest value at the same initial applied field employed in step (d),
- (i) establishing with the crest value for the virgin electrophotographic imaging member a fourth reference datum for dark decay crest value at the same final applied field employed in step (e),
- (j) determining the differential increase in dark decay between the third reference datum and the fourth reference datum to establish a differential increase in dark decay value for the virgin electrophotographic imaging member, and
- (k) comparing the differential increase in dark decay value of the virgin electrophotographic imaging member with the known differential increase in dark decay value to ascertain the projected microdefect levels of the virgin electrophotographic imaging member.

The motionless scanner is described in U.S. Pat. No. 5,175,503, the entire disclosure thereof being incorporated herein by reference. To conduct the DIDD and motionless scanner cycling tests described above, the photoreceptor sample was first coated with a gold electrode on the imaging surface. The sample was then connected to a DC power supply through a contact to the gold electrode. The sample was charged to a voltage by the DC power supply. A relay was connected in series with the sample and power supply. After 100 milliseconds of charging, the relay was opened to disconnect the power supply from the sample. The sample was dark rested for a predetermined time, then exposed to a light to discharge the surface voltage to the background level and thereafter exposed to more light to further discharge to the residual level. The same charge-dark and rest-erase cycle was repeated for a few cycles until a crest value of dark decay was reached. The sample surface voltage was measured with a non-contact voltage probe during this cycling period.

The duplicate photoconductive imaging members of all the above Examples were also tested for adhesive properties using a 180° (reverse) peel test technique. The 180° peel strength was determined by cutting a minimum of five 0.5 inch×6 inches imaging member samples from each of these Examples. For each sample, the charge transport layer is partially stripped from the test imaging member sample with the aid of a razor blade and then hand peeled to about 3.5 inches from one end to expose part of the underlying charge generating layer. The test imaging member sample is secured with its charge transport layer surface toward a 1 inch×6 inches×0.5 inch aluminum backing plate with the aid of two sided adhesive tape, 1.3 cm (½ inch) width Scotch® Magic Tape #810, available from 3M Company. At this condition, the anti-curl layer/substrate of the stripped segment of the test sample can easily be peeled away 180° from the sample to cause the adhesive layer to separate from the charge generating layer. The end of the resulting assembly opposite to the end from which the charge transport layer is not stripped is inserted into the upper jaw of an Instron

Tensile Tester. The free end of the partially peeled anti-curl/substrate strip is inserted into the lower jaw of the Instron Tensile Tester. The jaws are then activated at a 1 inch/min crosshead speed, a 2 inch chart speed and a load range of 200 grams to 180° peel the sample at least 2 inches. The load monitored with a chart recorder is calculated to give the peel strength by dividing the average load required for stripping the anti-curl layer with the substrate by the width of the test sample.

Although the electrical properties obtained for all the photoconductive imaging members of Examples I to XII had about equivalent photo-electrical characteristic, the imaging members of Examples II to XII having an invention adhesive interface layer (IFL) comprising polyvinyl carbazole (PVK) blending with Mor-Ester 49000, or polyarylate, or thermoplastic polyurethane (TPU), as shown in the following Table B, not only could provide reduced Charge deficient spots, as reflected in the reduction in DIDD values, but also gave significant layer adhesion bond strength enhancement compared to the result obtained for control imaging member counterpart of Comparative Example I

TABLE B

| EXAMPLE | ADHESIVE IFL LAYER | DIDD (VOLTS) | PEEL STRENGTH (GMS/CM) |
|---------|--------------------|--------------|------------------------|
| I       | 49000              | 415          | 5.3                    |
| II      | PVK/49K            | 180          | 5.6                    |
| III     | PVK/49K            | 118          | 5.5                    |
| IV      | PVK/49K            | 157          | 6.6                    |
| V       | PVK/49K            | 130          | 8.7                    |
| VI      | PVK/49K            | 125          | 10.2                   |
| VII     | PVK/49K            | 130          | 9.9                    |
| VIII    | PVK/Ardel          | 97           | >200.0                 |
| IX      | PVK/Ardel          | 57           | >200.0                 |
| X       | PVK/TPU            | 84           | 7.5                    |
| XI      | VK/TPU             | 22           | 7.3                    |
| XII     | PVK/TPU            | 161          | 6.8                    |

The data in the above table also show that adhesive interface layer modification through polymer blending with any of the selected polymer could significantly increase the peel strength of the layer. It is interesting to note that the presence or absence of hole transporting molecule of N,N'-diphenyl-N,N'-bis(3-methylphenyl)-1,1'-biphenyl-4,4'-diamine in the adhesive interface layer did not produce any impact on both the peel strength and the DIDD value of the resulting imaging member of Example VII.

While the embodiment disclosed herein is preferred, it will be appreciated from this teaching that various alternative, modifications, variations or improvements therein may be made by those skilled in the art, which are intended to be encompassed by the following claims.

What is claimed is:

- An electrophotographic imaging member comprising a support substrate having a two layered electrically conductive ground plane layer comprising a layer comprising zirconium over a layer comprising titanium, a hole blocking layer, an adhesive layer comprising a polymer blend comprising a carbazole polymer and a thermoplastic resin selected from the group consisting of copolyester, polyarylate and polyurethane in contiguous contact with said hole blocking layer, a charge generation layer comprising perylene or phthalocyanine pigment particles dispersed in a polycarbonate film forming binder in contiguous contact with said adhesive layer, and a hole transport layer, said hole transport layer being substantially non-absorbing in the spectral region at which the charge generation layer generates and injects photogenerated holes but being capable of

supporting the injection of photogenerated holes from said charge generation layer and transporting said holes through said charge transport layer.

2. An electrophotographic imaging member according to claim 1 wherein said carbazole polymer has the following structural formula:



(A)

wherein n, degree of polymerization, is number of between about 800 and about 6,000.

3. An electrophotographic imaging member according to claim 2 wherein said adhesive layer comprises between about 80 percent about 20 percent by weight of said carbazole polymer based on the total weight of said adhesive layer.

4. An electrophotographic imaging member according to claim 1 wherein said carbazole polymer has the following structural formula:



(B)

wherein n, degree of polymerization, is number of between about 900 and about 5,500.

5. An electrophotographic imaging member according to claim 1 wherein said carbazole polymer has the following structural formula:



(C)

wherein n, degree of polymerization, is number of between about 1,000 and about 5,000.

6. An electrophotographic imaging member according to claim 1 wherein said carbazole polymer has the following structural formula:



(D)

wherein n, degree of polymerization, is number of between about 1,000 and about 5,000.

7. An electrophotographic imaging member according to claim 1 wherein said film forming resin in said adhesive layer is a copolyester.

8. An electrophotographic imaging member according to claim 7 wherein said copolyester film forming resin in said

adhesive layer is a linear saturated copolyester reaction product of ethylene glycol with terephthalic acid, isophthalic acid, adipic acid and azelaic acid.

9. An electrophotographic imaging member according to claim 7 wherein said adhesive layer also comprises an arylamine charge transport molecule.

10. An electrophotographic imaging member according to claim 1 wherein said said film forming resin in said adhesive layer is a polyarylate.

11. An electrophotographic imaging member according to claim 10 wherein said polyarylate has the following repeating structural units:



12. An electrophotographic imaging member according to claim 1 wherein said said film forming resin in said adhesive layer is a polyurethane.

13. An electrophotographic imaging member according to claim 10 wherein said polyurethane has the following structural formula:



wherein:

R is diphenyl substituted methylene group or dicyclohexyl substituted methylene group,

R' is a straight alkyl chain hydrocarbon containing between 2 and 6 carbon atoms, and

J is, the degree of polymerization, between 90 and 500.

14. An electrophotographic imaging member according to claim 1 wherein said adhesive layer comprises between about 20 percent and about 80 by weight of said film forming resin, based on the total weight of said adhesive layer.

15. An electrophotographic imaging member according to claim 1 wherein said adhesive layer has a thickness of between about 0.03 micrometer and about 2 micrometers.

16. An electrophotographic imaging member according to claim 1 wherein said charge generation layer comprises a homogeneous vacuum sublimation deposited film of said perylene.

17. An electrophotographic imaging member according to claim 1 wherein said charge generation layer comprises a homogeneous vacuum sublimation deposited film of said phthalocyanine.

18. An electrophotographic imaging member according to claim 1 wherein said charge generation layer comprises said perylene dispersed as particles in a film forming binder.

19. An electrophotographic imaging member according to claim 18 wherein said film forming binder is poly(4,4'-diphenyl-1,1'-cyclohexane carbonate).

20. An electrophotographic imaging member according to claim 1 wherein said charge generation layer comprises said phthalocyanine is dispersed as particles in a film forming binder.

21. An electrophotographic imaging member according to claim 1 wherein said polycarbonate film forming binder in said charge generation layer comprises poly(4,4'-diphenyl-1,1'-cyclohexane carbonate).

22. An electrophotographic imaging member according to claim 1 wherein said two layered conductive ground plane layer has a thickness of between about 120 and about 300 angstroms.

23. An electrophotographic imaging member according to claim 1 wherein said zirconium layer has a thickness of at least about 60 angstroms.

24. An electrophotographic imaging member according to claim 1 wherein said hole blocking layer comprises a siloxane.

25. An electrophotographic imaging member according to claim 24 wherein said siloxane is an amino siloxane.

26. An electrophotographic imaging member according to claim 1 wherein said charge generation layer also comprises polyvinylcarbazole.

27. An electrophotographic imaging member according to claim 1 wherein said perylene is benzimidazole perylene.

28. An electrophotographic imaging member according to claim 1 wherein said charge generation layer also comprises between about 20 percent about 90 percent by volume of said benzimidazole perylene particles, based on the total volume of said charge generation layer.

\* \* \* \* \*